

3,057,725

SUBSTITUTED DISULFIDES AS ANTIFOGGANTS  
FOR SILVER HALIDE EMULSIONSArthur H. Herz and Norman W. Kalenda, Rochester, N.Y., assignors to Eastman Kodak Company, Rochester, N.Y., a corporation of New Jersey  
No Drawing. Filed July 17, 1959, Ser. No. 827,716  
16 Claims. (Cl. 96—109)

This invention relates to the stabilization of photographic silver halide emulsions, and more particularly, to a method of inhibiting development of spontaneous fog without adversely affecting the sensitivity of the photographic silver halide emulsions.

It is well known that photographic emulsions on storage tend to lose sensitivity and to become spontaneously developable without exposure to light. There is normally a detectable amount of the silver salt reduced during development in the areas where no exposure was given; this is commonly called "fog," and sometimes called "chemical fog" where it is necessary to distinguish between it and the effects of accidental exposure to radiation; in this invention, we are not concerned with the latter.

Fog depends both on the emulsion and the conditions of development; for a given emulsion it increases with the degree of development. With constant development conditions, it tends to increase with time, temperature and relative humidity of storage conditions; it is common practice to make accelerated tests of the stability of photographic emulsions by storage at increased temperature or humidity, or both. It is, of course, desirable to have emulsions as stable as possible under the conditions of high temperature and humidity which may occur in tropical climates, for example. Fog usually appears over the whole area of the sensitive coating, but when severe, it frequently is non-uniform. Fog may also be caused by exposure to chemicals, for example, hydrogen sulfide and other reactive sulfur compounds, hydrogen peroxide vapor, and strongly reducing materials. While antifoggants and stabilizers may protect, to some extent, against such effects, it is normally understood that antifoggants protect against spontaneous growth of fog during prolonged storage or storage at high temperatures and humidities, or during development to maximum contrast and speed, or both.

In emulsion technology, the use of certain organic disulfides as chemical sensitizers and stabilizers against incubation fog has been previously described. Unfortunately, many of these disulfides have properties which place them in more than one of the above categories. For example, cystine is known to exhibit both sensitizing and antifoggant behaviour. In like manner, the disulfides obtained from certain mercapto carboxylic acids, such as those described in Matthies et al. U.S. Patent 1,742,042, issued December 31, 1929, have primarily a sensitizing effect on photographic silver halide emulsions, with a much less marked effect upon the stability of the emulsions.

Because of the above facts, the use of such organic disulfides as antifoggants, offers practical disadvantages. Such disulfides having both sensitizing and some stabilizing activity cannot be employed in unsensitized or undersensitized emulsions. In fully sensitized, high-speed emulsions, the sensitizing or desensitizing disulfides, if they are to act as fog restrainers, must be used at narrow and controlled concentration levels, thus making their introduction into the emulsion, for example, by bathing, impractical.

It is, therefore, an object of our invention to provide a method of stabilizing photographic silver halide emulsions. Another object is to provide a method of stabiliz-

ing photographic silver halide emulsions without affecting to any material extent the sensitivity of the emulsions. Another object is to provide a method of stabilizing both unsensitized and sensitized emulsions, without introducing any substantial sensitizing or desensitizing effects. Still another object is to provide new organic disulfides and a method of preparation. Other objects will become apparent from a consideration of the following description and examples.

According to our invention, photographic silver halide emulsions can be stabilized and the development of spontaneous fog substantially inhibited by incorporating therein in certain organic disulfides.

The organic disulfides useful in practicing our invention comprise compounds selected from those represented by the following general formula:



wherein R and R<sub>1</sub> each represents a methylene group (which may or may not be substituted by hydrocarbon radicals, such as methyl, ethyl, phenyl, tolyl, etc., i.e., a hydrocarbon radical containing from 1 to 7 carbon atoms), m and n each represents a positive integer of from about 1 to 6 and X and Y each represent a radical:



or



wherein R<sub>2</sub> represents an alkoxy group (e.g., methoxyl, ethoxyl, etc.), an amine group (NH<sub>2</sub>), an alkylamino group (e.g., methylamino, ethylamino, etc.), a dialkylamino group (e.g., dimethylamino, diethylamino, etc.), or an —OM group wherein M represents a cation (e.g., hydrogen, sodium, potassium, ammonium, pyridinium, triethanolammonium, guanidinium, etc.), R<sub>3</sub> represents a hydrogen atom, an alkyl group (e.g., methyl, ethyl, propyl, isopropyl, butyl, etc.) or an aralkyl group (e.g., benzyl,  $\beta$ -phenylethyl, etc.), R<sub>4</sub> represents an acyl group (e.g., an acyl group of a carboxylic or sulfonic acid, such as acetyl, propionyl, butyryl, benzoyl, carbaniloyl, benzenesulfonyl, p-toluenesulfonyl, etc.), and R<sub>5</sub> represents a hydrogen atom, an alkyl group (e.g., methyl, ethyl, propyl, etc.), an aralkyl group (e.g., benzyl,  $\beta$ -phenylethyl, etc.), or an acyl group, such as those listed above

40 for R<sub>4</sub> (R<sub>4</sub> and R<sub>5</sub> may represent the same or different acyl groups).

Typical organic disulfides embraced by the above general formula include, for example, the following:



60 Potassium 1,1'-dimethyl-3,3'-dithiodipropanesulfonate or potassium 4,4'-dithiodi(2-butanonesulfonate)



- (7)  $\text{C}_6\text{H}_5\text{SO}_2\text{NHCH}_2\text{CH}_2-\text{S}-\text{S}-\text{CH}_2\text{CH}_2\text{NHSO}_2\text{C}_6\text{H}_5$   
2,2'-di(benzenesulfonamido) diethyldisulfide
- (8)  $\text{HOCH}_2\text{CH}_2-\text{S}-\text{S}-\text{CH}_2\text{CH}_2\text{OH}$   
2,2'-dihydroxydiethyldisulfide
- (9)  $\text{C}_6\text{H}_5\text{NHCOCH}_2\text{CH}_2-\text{S}-\text{S}-\text{CH}_2\text{CH}_2\text{OCOCH}_2\text{C}_6\text{H}_5$   
2,2'-di(phenylcarbamoyloxy) diethyldisulfide
- (10)  $\text{HOCH}_2\text{CH}_2\text{CH}_2-\text{S}-\text{S}-\text{CH}_2\text{CH}_2\text{CH}_2\text{OH}$   
3,3'-dihydroxydipropylsulfide
- (11)  $\text{C}_2\text{H}_5\text{OCH}_2\text{CH}_2-\text{S}-\text{S}-\text{CH}_2\text{CH}_2\text{OC}_2\text{H}_5$   
2,2'-dithoxydiethyldisulfide
- (12)  $\text{p-CH}_3\text{C}_6\text{H}_4\text{SO}_3\text{CH}_2\text{CH}_2-\text{S}-\text{S}-\text{CH}_2\text{CH}_2\text{O}_3\text{SC}_6\text{H}_4-\text{CH}_3(\text{p})$   
2,2'-di(p-toluenesulfonyloxy) diethyldisulfide
- (13)  $\text{C}_6\text{H}_5\text{COOCH}_2\text{CH}_2-\text{S}-\text{S}-\text{CH}_2\text{CH}_2\text{OOC-C}_6\text{H}_5$   
2,2'-dibenzoyldiethyldisulfide
- (14)  $\text{CH}_3\text{COOCH}_2\text{CH}_2-\text{S}-\text{S}-\text{CH}_2\text{CH}_2\text{OOCCH}_3$   
2,2'-diacetoxydiethyldisulfide
- (15)  $\text{H}_2\text{NSO}_2\text{CH}_2\text{CH}_2-\text{S}-\text{S}-\text{CH}_2\text{CH}_2\text{SO}_2\text{NH}_2$   
2,2'-disulfonamidoethyldisulfide

For the purpose of inhibiting fog formation, the disulfides of our invention can be added to the emulsion during the process of manufacture in order to avoid loss of sensitivity and to inhibit the growth of fog with passage of time under nonideal conditions of storage.

An aqueous or organic solution of the disulfides of our invention when added at suitable concentration to unsensitized, chemically sensitized, or optically sensitized photographic emulsions does not appreciably affect the sensitometric values for sensitivity and fog when measurements are made soon after coating. When sensitometric measurements are made at appreciable intervals of time, at elevated temperatures and dry or somewhat humid conditions, the disulfides of our invention do stabilize speed and maintain fog at a low level.

The preparation of silver halide emulsions involves three separations: (1) the emulsification and digestion or ripening of the silver halide, (2) the freeing of the emulsion from excess soluble salts, usually by washing, and (3) the second digestion or after-ripening to obtain increased sensitivity (Mees, "The Theory of the Photographic Process" (1942)). We prefer to add the fog-inhibiting agents after the final digestion or after-ripening, although they can advantageously be added prior to digestion.

If desired, the disulfides of our invention can be incorporated in the emulsions without adverse effects by bathing techniques known to those skilled in the art.

The photographic emulsions used in practicing our invention are of the developing-out type.

The emulsions can be chemically sensitized by any of the accepted procedures. The emulsions can be digested with naturally active gelatin, or sulfur compounds can be added such as those described in Sheppard U.S. Patent 1,574,944, issued March 2, 1926; Sheppard et al. U.S. Patent 1,623,499, issued April 5, 1927, and Sheppard et al. U.S. Patent 2,410,689, issued November 5, 1946.

The emulsions can also be treated with salts of the noble metals such as ruthenium, rhodium, palladium, iridium, and platinum. Representative compounds are ammonium chloropalladate, potassium chloroplatinate, and sodium chloropalladite, which are used for sensitizing in amounts below that which produces any substantial fog inhibition, as described in Smith and Trivelli U.S. Patent 2,448,060, issued August 31, 1948.

The emulsions can also be chemically sensitized with gold salts as described in Waller et al. U.S. Patent 2,399,083, issued April 23, 1946, or stabilized with gold salts as described in Damschroder U.S. Patent 2,597,856, issued May 27, 1952, and Yutzy and Leermakers U.S. Patent

2,597,915, issued May 27, 1952. Suitable compounds are potassium chloroaurite, potassium aurithiocyanate, potassium chloroaurate, auric trichloride and 2-aurosulfo-benzothiazole methochloride.

5 The emulsions can also be chemically sensitized with reducing agents such as stannous salts (Carroll U.S. Patent 2,487,850, issued November 15, 1949), polyamines, such as diethyl triamine (Lowe and Jones U.S. Patent 2,518,698, issued August 15, 1950), polyamines, such as 10 spermine (Lowe and Allen U.S. Patent 2,521,925, issued September 12, 1950), or bis(β-aminoethyl)sulfide and its water-soluble salts (Lowe and Jones U.S. Patent 2,521,926, issued September 12, 1950).

The emulsions can also be optically sensitized with 15 cyanine and merocyanine dyes, such as those described in Brooker U.S. Patents 1,846,301, issued February 23, 1932; 1,846,302, issued February 23, 1932; and 1,942,854, issued January 9, 1934; White U.S. Patent 1,990,507, issued February 12, 1935; Brooker and White U.S. Patents 2,112,140, issued March 22, 1938; 2,165,338, issued July 11, 1939; 2,493,747, issued January 10, 1950, and 2,739,964, issued March 27, 1956; Brooker and Keyes U.S. Patent 2,493,748, issued January 10, 1950; Sprague U.S. Patents 2,503,776, issued April 11, 1950, and 2,519,-

25 001, issued August 15, 1950; Heseltine and Brooker U.S. Patent 2,666,761, issued January 19, 1954; Heseltine U.S. Patent 2,734,900, issued February 14, 1956; Van Lare U.S. Patent 2,739,149, issued March 20, 1956; and Kodak Limited British Patent 450,958, accepted July 15, 1936.

30 The emulsions may also contain speed-increasing compounds of the quaternary ammonium type of Carroll U.S. Patent 2,271,623, issued February 3, 1942; Carroll and Allen U.S. Patent 2,288,226, issued June 30, 1942; and Carroll and Spence U.S. Patent 2,334,864, issued November 23, 1943; and the polyethylene glycol type of Carroll and Beach U.S. Patent 2,708,162, issued May 10, 1955, and the thioether compounds of Graham and Sagal U.S. application Serial No. 779,839, filed December 12, 1958, and the Dann and Gates U.S. application Serial No. 797,-

40 577, filed March 6, 1959.

The emulsions may contain a suitable gelatin plasticizer such as glycerin; a dihydroxy alkane such as 1,5-pentane diol as described in Milton and Murray U.S. application Serial No. 588,951, filed June 4, 1956; an ester of an ethylene bis-glycolic acid such as ethylene bis(methyl glycolate) as described in Milton U.S. application Serial No. 662,564, filed May 31, 1957; bis(ethoxy diethylene glycol) succinate as described in Gray U.S. application Serial No. 604,333, filed August 16, 1956, or a polymeric hydro-

50 50 sol as results from the emulsion polymerization of a mixture of an amide of an acid of the acrylic acid series, an acrylic acid ester and a styrene-type compound as described in Tong U.S. Patent 2,852,386, issued September 16, 1958. The plasticizer may be added to the emulsion before or after the addition of a sensitizing dye, if used.

The emulsions may be hardened with any suitable hardener for gelatin such as formaldehyde; a halogen-substituted aliphatic acid such as mucobromic acid as described in White U.S. Patent 2,080,019, issued May 11, 1937; a 60 compound having a plurality of acid anhydride groups such as 7,8-diphenylbicyclo(2,2,2)-7-octene-2,3,5,6-tetra-carboxylic dianhydride, or a dicarboxylic or a disulfonic acid chloride such as terephthaloyl chloride or naphthalene-1,5-disulfonyl chloride as described in Allen and Carroll U.S. Patents 2,725,294 and 2,725,295, both issued November 29, 1955; a cyclic 1,2-diketone such as cyclopentane-1,2-dione as described in Allen and Byers U.S. Patent 2,725,305, issued November 29, 1955; a bisester of methane-sulfonic acid such as 1,2-di-(methane-sulfonyloxy)-70 ethane as described in Allen and Laakso U.S. Patent 2,726,162, issued December 6, 1955; 1,3-dihydroxymethyl-benzimidazol-2-one as described in July, Knott and Pollak U.S. Patent 2,732,316, issued January 24, 1956; a dialdehyde or a sodium bisulfite derivative thereof, the aldehyde groups of which are separated by 2-3 carbon atoms, such

as  $\beta$ -methyl glutaraldehyde bis-sodium bisulfite as described in Allen and Burness U.S. Patent application Serial No. 556,031, filed December 29, 1955; a bis-aziridine carboxamide such as trimethylene bis(1-aziridine carboxamide) as described in Allen and Webster U.S. patent application Serial No. 599,891, filed July 25, 1956; or 2,3-dihydroxy dioxane as described in Jeffreys U.S. Patent 2,870,013, issued January 20, 1959.

The emulsions may contain a coating aid such as saponin; a lauryl or oleyl monoether of polyethylene glycol as described in Knox and Davis U.S. Patent 2,831,766, issued April 22, 1958; a salt of a sulfated and alkylated polyethylene glycol ether as described in Knox and Davis U.S. Patent 2,719,087, issued September 27, 1955; an acylated alkyl taurine such as the sodium salt of N-oleoyl-N-methyl taurine as described in Knox, Twardokus and Davis U.S. Patent 2,739,891, issued March 27, 1956; the reaction product of a dianhydride of tetracarboxybutane with an alcohol or an aliphatic amine containing from 8 to 18 carbon atoms which is treated with a base, for example, the sodium salt of the monoester of tetracarboxybutane as described in Knox, Stenberg and Wilson U.S. Patent 2,843,487, issued July 15, 1958; a water-soluble maleopimarate or a mixture of a water-soluble maleopimarate and a substituted glutamate salt as described in Knox and Fowler U.S. Patent 2,823,123, issued February 11, 1958; an alkali metal salt of a substituted amino acid such as disodium N-(carbo-p-tert. octylphenoxy)pentaoxy glutamate as described in Knox and Wilson U.S. patent application Serial No. 600,679, filed July 30, 1956; or a sulfosuccinamate such as tetrasodium N-(1,2-dicarboxyethyl)-N-octadecyl sulfosuccinamate or N-lauryl disodium sulfosuccinamate as described in Knox and Stenberg U.S. patent application Serial No. 691,125, filed October 21, 1957.

The addenda which we have described may be used in various kinds of photographic emulsions. In addition to being useful in X-ray and other nonoptically sensitized emulsions they may also be used in orthochromatic, panchromatic, and infrared sensitive emulsions. They may be added to the emulsion before or after any sensitizing dyes which are used. Various silver salts may be used as the sensitive salts such as silver bromide, silver iodide, silver chloride, or mixed silver halides such as silver chlorobromide or silver bromoiodide. The agents may be used in emulsions intended for color photography, for example, emulsions containing color-forming couplers or emulsions to be developed by solutions containing couplers or other color-generating materials, emulsions of the mixed-packet type, such as described in Godowsky U.S. Patent 2,698,794, issued January 4, 1955; or emulsions of the mixed-grain type, such as described in Carroll and Hanson U.S. Patent 2,592,243, issued April 8, 1952. These agents can also be used in emulsions which form latent images predominantly on the surface of the silver halide crystal or in emulsions which form latent images predominantly inside the silver halide crystal, such as those described in Davey and Knott U.S. Patent 2,592,250, issued April 8, 1952.

These may also be used in emulsions intended for use in diffusion transfer processes which utilize the undeveloped silver halide in the nonimage areas of the negative to form a positive by dissolving the undeveloped silver halide and precipitating it on a receiving layer in close proximity to the original silver halide emulsion layer. Such processes are described in Rott U.S. Patent 2,352,014, issued June 20, 1944, and Land U.S. Patents 2,584,029, issued January 29, 1952, 2,698,236, issued December 28, 1954, and 2,543,181, issued February 27, 1951; and Yackel et al. U.S. patent application Serial No. 586,705, filed May 23, 1956. They may also be used in color transfer processes which utilize the diffusion transfer of an image-wise distribution of developer, coupler or dye, from a light-sensitive layer to a second layer, while the two layers are in close proximity to one another. Color

processes of this type are described in Land U.S. Patents 2,559,643, issued July 10, 1951, and 2,698,798, issued January 4, 1955; Land and Rogers Belgian Patents 554,933 and 554,934, granted August 12, 1957; International Polaroid Belgian Patents 554,212, granted July 16, 1957, and 554,935, granted August 12, 1957; Yutzy U.S. Patent 2,756,142, granted July 24, 1956, and Whitmore and Mader U.S. patent application Serial No. 734,141, filed May 9, 1958.

10 In the preparation of the silver halide dispersions employed for preparing silver halide emulsions, there may be employed as the dispersing agent for the silver halide in its preparation, gelatin or some other colloidal material such as colloidal albumin, a cellulose derivative, or 15 a synthetic resin, for instance, a polyvinyl compound. Some colloids which may be used are polyvinyl alcohol or a hydrolyzed polyvinyl acetate as described in Lowe U.S. Patent 2,286,215, issued June 16, 1942; a far hydrolyzed cellulose ester such as cellulose acetate hydrolyzed to an acetyl content of 19-26% as described in U.S. Patent 2,327,808 of Lowe and Clark, issued August 24, 1943; a water-soluble ethanolamine cellulose acetate as described in Yutzy U.S. Patent 2,322,085, issued June 15, 1943; a polyacrylamide having a combined acrylamide content of 30-60% and a specific viscosity of 0.25-1.5 on an imidized polyacrylamide of like acrylamide content and viscosity as described in Lowe, Minsk and Kenyon U.S. Patent 2,541,474, issued February 13, 1951; zein as described in Lowe U.S. Patent 2,563,791, issued August 7, 1951; a vinyl alcohol polymer containing urethane carboxylic acid groups of the type described in Unruh and Smith U.S. Patent 2,768,154, issued October 23, 1956; or containing cyano-acetyl groups such as the vinyl alcohol-vinyl cyanoacetate copolymer as described in Unruh, 20 Smith and Priest U.S. Patent 2,808,331, issued October 1, 1957; or a polymeric material which results from polymerizing a protein or a saturated acylated protein with a monomer having a vinyl group as described in U.S. Patent 2,852,382, of Illingsworth, Dann and Gates, issued 25 September 16, 1958.

If desired, compatible mixtures of two or more of these colloids may be employed for dispersing the silver halide in its preparation. Combinations of these sensitizers, hardeners, etc., may be used.

45 The organic disulfides useful in practicing our invention can be added to the photographic emulsions prior to the final digestion, if desired. Generally, these compounds can be added from a substantially neutral solution so that the pH of the emulsion is not disturbed. In 50 the case of compounds containing free sulfonic acid groups, this means that these sulfonic acid groups may be at least partially neutralized. However, where it is desired to stabilize an acidic emulsion, it is obviously not necessary that the antifoggant be added from substantially neutral solutions. Since the disulfides of our invention can be added to the emulsions in such small 55 quantities, it is apparent that they will generally have no adverse effect upon the pH of the emulsions. Many of the organic disulfides useful in practicing our invention can be added to the emulsions in the form of substantially neutral aqueous solutions. If a particular disulfide does not have sufficient solubility in water, addition to the emulsion can be made in the form of a water-miscible organic solvent, such as methanol, ethanol, di-60 oxane, pyridine, etc.

65 The amount of disulfide compound added to the emulsions of our invention can be varied, depending upon the particular emulsion, the silver halide content of the emulsion, etc. In general, we have found that from about 0.1 to 15.0 grams of disulfide per mole of silver halide can advantageously be employed in our invention. One of the outstanding advantages of the disulfides of 70 our invention, as compared with the disulfides which have been previously described in the prior art, is that they can be used in quite substantial quantities without intro-75

ducing serious desensitizing effects. Moreover, as indicated above, the disulfides useful in our invention advantageously have little or no sensitizing action of their own, and hence, they can be used to stabilize emulsions which have already been finished to their optimum or near-optimum speeds. Thus, addition of our compounds to such finished emulsions does not result in any substantial desensitizing effect, such as might ordinarily be expected.

The following examples will serve to illustrate the useful stabilizing effect of many of the organic disulfides useful in practicing our invention. A series of coatings was made on ordinary photographic film support, such as cellulose acetate, of an ordinary photographic high-speed bromiodide emulsion, to which had been added one of the organic disulfides of our invention at the concentration shown in the following table. The compounds were added from substantially neutral solutions and comparisons were made with an identical batch of emulsion which contained no antifoggant compound. After coating each series of emulsions on a cellulose acetate support, the emulsions were dried and then exposed on an intensity scale sensitometer (Kodak Type Ib) and developed for about 4 minutes at 68° F. in a developer having the following composition:

|                                      |       |      |
|--------------------------------------|-------|------|
| Water, about 125° C. (50° C.)        | cc    | 500  |
| Kodak Elon developing agent          | grams | 2.0  |
| Kodak sodium sulfite, desiccated     | do    | 90.0 |
| Kodak hydroquinone                   | do    | 8.0  |
| Kodak sodium carbonate, monohydrated | do    | 52.5 |
| Kodak potassium bromide              | do    | 5.0  |
| Cold water to make 1.0 liter.        |       |      |

Fresh tests and incubation tests (one week at 120° F., constant relative humidity of about 50%, and in some cases for two weeks under the same conditions) were also run for the same emulsion series with development under the same conditions. The relative speed and fog for each of the series coatings were then measured, the speed being determined at a point about 0.3 density above fog.

In the following table the compound numbers correspond to the numbers used above for the specific disulfides. In each coating series, the same emulsion batch was used, although different emulsion batches were used for some of the coating numbers identified in the coating table. Wherever a different emulsion batch was used, a new control series was run for that batch to show the degree of improvement obtained. The results of these coating series are given in the following table:

| Coating No. | Addendum Compound No. (g./mol. AgX) | Fresh Test |     | One Week Incubation Test |     | Two Week Incubation Test |  |
|-------------|-------------------------------------|------------|-----|--------------------------|-----|--------------------------|--|
|             |                                     | Speed      | Fog | Speed                    | Fog | Fog                      |  |
|             |                                     |            |     |                          |     |                          |  |
| 1. (a)      | None                                | 100        | .08 | 139                      | .22 | .62                      |  |
| (b)         | 1 (11.4)                            | 100        | .09 | 136                      | .15 | .48                      |  |
| (c)         | 3 (12.3)                            | 100        | .07 | 158                      | .11 | .25                      |  |
| 2. (d)      | None                                | 100        | .13 | 87                       | .31 | .66                      |  |
| (e)         | 2 (6.3)                             | 112        | .11 | 103                      | .21 | .40                      |  |
| 3. (f)      | None                                | 100        | .17 | 94                       | .22 | .49                      |  |
| (g)         | 6 (1.1)                             | 94         | .16 | 83                       | .14 | .16                      |  |
| (h)         | 7 (1.3)                             | 107        | .14 | 105                      | .15 | .22                      |  |
| 4. (i)      | None                                | 100        | .11 | 155                      | .29 | .89                      |  |
| (j)         | 8 (0.48)                            | 85         | .11 | 141                      | .21 | .50                      |  |
| (k)         | 9 (1.2)                             | 87         | .09 | 162                      | .14 | .40                      |  |
| (l)         | 9 (3.0)                             | 76         | .10 | 132                      | .12 | .29                      |  |
| 5. (m)      | None                                | 100        | .17 | 82                       | .25 | .49                      |  |
| (n)         | 5 (0.72)                            | 107        | .18 | 102                      | .16 | .21                      |  |

The disulfides useful in stabilizing emulsions according to our invention can be obtained by methods which have been previously described in the prior art. For example, the disulfides of Formula IA can be obtained by

simple oxidation of the corresponding mercapto-substituted sulfonic acid or derivative. Oxidation can conveniently be accomplished by simply contacting the mercapto derivative with an oxidizing agent, such as hydrogen peroxide, sodium perchlorate, etc. The following examples will serve to illustrate this technique.

#### EXAMPLE A

##### *Potassium 3,3'-Dithiodipropanesulfonate*

10 Guanidinium 3-mercaptopropanesulfonate (1 mol., 6.05 g.) was dissolved in 14 ml. water and passed through an Amberlite IR-120 (ion exchange resin) column operating in the acid phase. The column was washed with water (ca. 85 ml.) until the eluate was neutral to indicator paper. The eluate, containing 3-mercaptopropanesulfonic acid, was treated with 30% hydrogen peroxide (1/2 mol. + 12%, 1.8 g.) and allowed to stand at room temperature for 3 hours. The solution was neutralized with aqueous potassium hydroxide, and water was removed in vacuo. The residue was washed well with ether and dried. After two recrystallizations from aqueous ethanol, the yield of purified potassium 3,3'-dithiodipropanesulfonate was 2.68 g. (49%).

Analysis.—Calcd. for  $C_6H_{12}O_6S_2K_2$ : C, 18.6; H, 3.1; S, 33.2. Found: C, 18.7; H, 3.1; S, 33.6.

#### EXAMPLE B

##### *Potassium 4,4'-Dithiodibutanesulfonate*

30 Guanidinium 4-mercaptopbutanesulfonate (1 mol., 7.00 g.) was dissolved in 15 ml. water and passed through an Amberlite IR-120 column operating in the acid phase. The column was washed with water until the eluate was neutral to indicator paper. The eluate, containing 4-mercaptopbutanesulfonic acid, was treated with 30% hydrogen peroxide (1/2 mol., 1.8 g.), and allowed to stand at room temperature for one day. The solution was neutralized with aqueous potassium hydroxide, and water was removed in vacuo. The residue was stirred with ethanol, filtered off, and dried. After two recrystallizations from aqueous ethanol, the yield of purified potassium 4,4'-dithiodibutanesulfonate was 4.36 g. (69%).

Analysis.—Calcd. for  $C_8H_{16}O_6S_2K_2$ : C, 23.2; H, 3.9; S, 30.9. Found: C, 23.1; H, 4.0; S, 20.6.

#### EXAMPLE C

##### *Potassium 4,4'-Dithiodi(2-Butanesulfonate)*

50 Guanidinium 4-mercaptop-2-butanesulfonate (1 mol., 10.00 g.) was dissolved in 100 ml. water and passed through an Amberlite IR-120 column operating in the acid phase. The column was washed with water until the eluate was neutral to indicator paper. The eluate, containing 4-mercaptop-2-butanesulfonic acid, was treated with 30% hydrogen peroxide (1/2 mol., 2.5 g.) and allowed to stand at room temperature three days. The solution was neutralized with aqueous potassium hydroxide, and concentrated in vacuo to a paste. The paste was stirred with ethanol, and the solid was filtered off and dried. After two recrystallizations from aqueous ethanol, the yield of purified potassium 4,4'-dithiodi(2-butanesulfonate) was 5.53 g. (61%).

Analysis.—Calcd. for  $C_8H_{16}O_6S_4K_2$ : C, 23.2; H, 3.9; S, 30.9. Found: C, 23.7; H, 3.8; S, 31.0.

#### EXAMPLE D

##### *Guanidinium 4,4'-Dithiodi(2-Butanesulfonate)*

70 Guanidinium 4-mercaptop-2-butanesulfonate (1 mol., 5.00 g.) was dissolved in 50 ml. water and the solution was made slightly alkaline with aqueous ammonia. A catalytic amount (ca. 0.05 g.) of ferrous sulfate was added, and a dark brown solution resulted. The solution was stirred and gradually 30% hydrogen peroxide (1/2 mol. + 10%, 1.4 g.) was added. When addition was complete, the solution turned colorless. Iron hydroxides

were filtered off, and the filtrate was taken to near dryness in vacuo. The solid was filtered from a very small amount of water which remained, and dried. After two recrystallizations from methanolic chloroform the yield of purified guanidinium 4,4'-dithiodi(2-butanesulfonate) was 3.28 g. (66%), M.P. 231-3° C.

*Analysis.*—Calcd. for  $C_{10}H_{28}N_6O_6S_4$ : C, 26.3; H, 6.2; S, 28.1. Found: C, 26.3; H, 6.2; S, 28.2.

The 3-mercaptopropanesulfonic acid salts and corresponding 4-mercaptopbutanesulfonic acid salt were previously described by Schramm, Lemaire, and Karlson, JACS, 77, 6231 (1955).

The disulfides of Formula IB can be prepared by simply acylating the corresponding amino compound. Acylation can be accomplished by merely contacting the corresponding amino-disulfide with an acylhalide. In like manner, the disulfides of Formula IC, wherein  $R_5$  represents an acyl group, can be obtained by merely acylating the corresponding compounds of Formula IC, wherein  $R_5$  represents a hydrogen atom. Techniques of acylation are well known to those skilled in the art and no particular knowledge is required in order to acylate the amino or hydroxyl-substituted organic disulfides.

What we claim as our invention and desired secured by Letters Patent of the United States is:

1. A photographic silver halide emulsion stabilized with a water-soluble compound selected from the class consisting of those represented by the following general formula:



wherein R represents an alkylene group having from 1 to about 6 carbon atoms and X represents a radical selected from the class consisting of  $-SO_2R_2$ ,



and  $-OR_5$ , wherein  $R_2$  represents a member selected from the class consisting of an alkoxy group having from 1 to about 6 carbon atoms and a  $-OM$  group wherein M represents a cation,  $R_3$  represents a member selected from the class consisting of a hydrogen atom and an alkyl group having from 1 to about 6 carbon atoms,  $R_4$  represents an acyl group of an organic acid selected from the class consisting of carboxylic acids and sulfonic acids, and  $R_5$  represents a member selected from the class consisting of a hydrogen atom, an alkyl group having from 1 to about 6 carbon atoms and an acyl group of an organic acid selected from the class consisting of carboxylic acids and sulfonic acids.

2. A photographic silver halide emulsion stabilized with a water-soluble compound selected from the class consisting of those represented by the following general formula:



wherein R represents an alkylene group having from 1 to about 6 carbon atoms, and  $R_2$  represents a member selected from the class consisting of an alkoxy group having from 1 to about 6 carbon atoms and a  $-OM$  group wherein M represents a cation.

3. A photographic silver halide emulsion stabilized with a water-soluble compound selected from the class consisting of those represented by the following general formula:



wherein R represents an alkylene group having from 1 to about 6 carbon atoms,  $R_3$  represents a member selected from the class consisting of a hydrogen atom, an alkyl group having from 1 to about 6 carbon atoms, and  $R_4$  represents an acyl group of an organic acid selected from the class consisting of carboxylic acids and sulfonic acids.

4. A photographic silver halide emulsion stabilized with a water-soluble compound selected from the class

consisting of those represented by the following general formula:



5. A photographic silver halide emulsion stabilized with a water-soluble compound selected from the class consisting of those represented by the following general formula:



wherein  $m$  represents a positive integer of from about 1 to 6 and  $R_2$  represents a member selected from the class consisting of an alkoxy group having from 1 to about 6 carbon atoms and a  $-OM$  group wherein M represents a cation.

6. A photographic silver halide emulsion stabilized with a water-soluble compound selected from the class consisting of those represented by the following general formula:



wherein  $m$  represents a positive integer of from about 1 to 6,  $R_3$  represents a member selected from the class consisting of a hydrogen atom and an alkyl group having from 1 to about 6 carbon atoms and  $R_4$  represents an acyl group of an organic acid selected from the class consisting of carboxylic acids and sulfonic acids.

7. A photographic silver halide emulsion stabilized with a water-soluble compound selected from the class consisting of those represented by the following general formula:



wherein  $m$  represents a positive integer of from about 1 to 6 and  $R_5$  represents a member selected from the class consisting of a hydrogen atom, an alkyl group having from 1 to about 6 carbon atoms and an acyl group of an organic acid selected from the class consisting of carboxylic acids and sulfonic acids.

8. A photographic silver halide emulsion stabilized with a water-soluble compound selected from the class consisting of those represented by the following general formula:



wherein R represents an alkylene group having from 1 to about 6 carbon atoms and M represents a cation.

9. A photographic silver halide emulsion stabilized with a water-soluble compound selected from the class consisting of those represented by the following general formula:



wherein R represents an alkylene group having from 1 to about 6 carbon atoms and  $R_4$  represents an acyl group of an organic acid selected from the class consisting of carboxylic acids and sulfonic acids.

10. A photographic silver halide emulsion stabilized with a water-soluble compound selected from the class consisting of those represented by the following general formula:



wherein R represents an alkylene group having from 2 to about 6 carbon atoms.

11. A photographic silver halide emulsion stabilized with a water-soluble compound selected from the class

consisting of those represented by the following general formula:



wherein R represents an alkylene group having from 2 to about 6 carbon atoms and R<sub>5</sub> represents an acyl group of an organic acid selected from the class consisting of carboxylic acids and sulfonic acids.

12. A photographic silver halide emulsion stabilized with potassium 3,3'-dithiodipropanesulfonate. 10

13. A photographic silver halide emulsion stabilized with N,N'-dibenzoyl-2,2'-diaminodithyldisulfide. 5

14. A photographic silver halide emulsion stabilized with 2,2'-dihydroxydithyldisulfide.

15. A photographic silver halide emulsion stabilized with 2,2'-di(phenylcarbamyl)oxy)dithyldisulfide.

16. A photographic silver halide emulsion stabilized with 2,2'-di(benzenesulfonamido)dithyldisulfide.

References Cited in the file of this patent

UNITED STATES PATENTS

- |    |           |             |       |               |
|----|-----------|-------------|-------|---------------|
| 10 | 2,438,716 | Mueller     | ----- | Mar. 30, 1948 |
|    | 2,440,206 | Mueller     | ----- | Apr. 20, 1948 |
|    | 2,739,060 | Lowe et al. | ----- | Mar. 20, 1956 |